

# United States Patent

[19]

Rushmere

[11] 3,855,085

[45] Dec. 17, 1974

[54] ACID ZINC ELECTROPLATING  
ELECTROLYTE, PROCESS AND ADDITIVE

3,669,854 6/1972 Harbulak ..... 204/55 R  
3,694,330 9/1972 Korpiun ..... 204/55 R  
3,758,386 9/1973 Chan ..... 204/55 R

[75] Inventor: John Derek Rushmere, Wilmington, Del.

[73] Assignee: E. I. du Pont de Nemours and Company, Wilmington, Del.

[22] Filed: June 14, 1973

[21] Appl. No.: 369,815

*Primary Examiner*—G. L. Kaplan

[52] U.S. Cl. ..... 204/55 R, 204/DIG. 2

[51] Int. Cl. ..... C23b 5/12, C23b 5/46

[58] Field of Search ..... 204/55 R, 55 Y, 43 Z, 44, 204/DIG. 2

## [56] References Cited

### UNITED STATES PATENTS

3,594,291 7/1971 Todt et al. ..... 204/55 R

## [57] ABSTRACT

Bright zinc electroplates can be deposited from electrolytes containing zinc chloride, ammonium chloride, and an addition agent comprising a mixture of certain nonionic polyoxyethylene compounds, certain ketones and certain carboxylic acids.

30 Claims, No Drawings

# ACID ZINC ELECTROPLATING ELECTROLYTE, PROCESS AND ADDITIVE

## BACKGROUND OF THE INVENTION

This invention relates to the deposition of bright zinc 5 electroplate, and more particularly to the electrodeposition of such plate from acid electrolytes.

It is presently recognized that there are certain advantages to being able to plate bright zinc electrodeposits from acid rather than conventional basic cyanide baths. These advantages include the ability to plate cast 10 iron and carbonitrided steel as well as the avoidance of problems associated with the disposal of toxic cyanide wastes. Thus, a number of processes have been proposed recently for electroplating bright zinc from acid 15 baths which do not contain cyanides.

In operating such acid zinc processes, certain additives are required to obtain bright plate over a commercially operable range of current densities and improved processes, and additives are always desirable to extend this range of operating current densities thus permitting 20 more flexibility in plating, especially in the plating of objects with complex surface configurations.

Certain polyoxyethylene compounds and certain ketone compounds have been proposed for use in bright acid zinc electroplating, usually in combination with other additives. For example, U.S. Pat. No. 3,594,291 — Todt et al. describes the use of certain ketones with N-polyvinyl pyrrolidone as brighteners in such baths, 25 although the plate produced is not truly bright at high current densities. U.S. Pat. No. 3,694,330 — Korpiun et al. and generally corresponding British Pat. No. 1,149,106 disclose the use, along with an aromatic carbonyl compound and ammonium chloride, of a non-ionogenic, surface active polyoxyethylene compound. Suitable aromatic carbonyl compounds are said to include carboxylic acids, carboxylic acid esters, aldehydes and ketones. However, the disclosures do not teach the combined use of both carboxylic acids and 30 ketones but rather the use of them individually as equivalents. The bright plating range is also limited to 10 to 50 a./ft.<sup>2</sup>, although the range below 10 a./ft.<sup>2</sup> is particularly desirable for commercial barrel plating operations.

U.S. Pat. No. 3,669,854 — Harbulak teaches bright acid zinc electroplating using as additives polyethers and at least one nonaromatic  $\alpha,\beta$ -unsaturated carbonyl compound. Harbulak also discloses the use of citric acid as a bath component in addition to the polyoxyethylene compound and a ketone. However, the function of the citric acid is that of a complexing agent rather than that of a brightener. The citric acid maintains the zinc in solution at pH's above 5.5, preventing the precipitation of insoluble zinc salts.

## SUMMARY OF THE INVENTION

The present invention, in certain of its embodiments, provides compositions for acid zinc electrolytic plating baths and additives for such baths, as well as methods for using such baths.

The plating bath compositions of the invention comprise an aqueous bath composition containing at least one zinc compound providing zinc ions for electroplating zinc, a source of chloride ion, at least one nonionic polyoxyethylene compound, at least one ketone, and at least one carboxylic acid, wherein

said polyoxyethylene compound is selected from compounds of the formula



wherein  $n + m \geq 10$ ,  $x = 1$  or  $2$ , derived from a reaction of oxyethylene with a polyol selected from the group consisting of

2,4,7,9-tetramethyl-5-decyne-4,7 diol,

polyoxypropylene glycol of molecular weight at least about 900, and  
 $\text{N},\text{N}',\text{N}',\text{N}'$ -tetrakis(polyoxypropylene glycol) ethylene diamine of molecular weight at least about 500,

and wherein R is defined by the selected polyol; said ketone is selected from the group consisting of

4-phenyl-3-buten-2-one (benzalacetone),  
 4-(4-methoxyphenyl)-3-buten-2-one (anisalacetone),

4,(3,4-dimethoxyphenyl)-3-buten-2-one (veratralacetone),

4-(3,4-methylenedioxyphenyl)-3-buten-2-one (piperonalacetone), and

4-(2-furyl)-3-buten-2-one (furfuralacetone); and said carboxylic acid is selected from the group consisting of

benzoic acid,

cinnamic acid,

2-furylacrylic acid, and

nicotinic acid.

The polyoxyethylene - 2,4,7,9-tetramethyl-5-decyne-4,7 diol is sold under the name "Surfynol" by Air Products and Chemicals, Inc., of Wayne, Pa. The polyoxyethylene - polyoxypropylene glycol is sold under the name "Pluronic" by BASF Wyandotte Corp. of Wyandotte, Michigan. The polyoxyethylene-N,N',N',N'-tetrakis(polyoxypropylene glycol) ethylene diamine is sold under the name "Tetronic" by BASF Wyandotte Corp.

The bath is preferably operated at a pH between 3.5 and 6.1. The preferred pH range for optimum brightness and operability is 5 to 6. Zinc deposits of acceptable commercial quality can be obtained over the temperature range of 15° to 40°C., and the preferred operating temperature range is 20° to 35°C. The preferred range of zinc metal content in the bath is 30 to 60 g./l., preferably added as zinc chloride. For best results, the bath should have a total chloride ion content of 150 to 190 g./l., with the major portion (over 50% by weight) of the chloride, other than that derived from zinc chloride, added in the form of ammonium chloride.

The concentration ranges of the brightening additives in the bath are as follows: polyoxyethylene compounds 0.05 to 20 g./l., preferably 2 to 10 g./l., ketone: 0.05 to 2 g./l., preferably 0.1 to 0.5 g./l.; carboxylic acid: 0.05 to 20 g./l., preferably 1 to 6 g./l. In the addition agent of the invention used to prepare and maintain the baths, the concentration ranges of the brightening additives are: polyoxyethylene compounds: 10 to 400 g./l., preferably 20 to 50 g./l.; ketone: 10 to 200 g./l., preferably 20 to 50 g./l.; carboxylic acid: 10 to 200 g./l., preferably 20 to 50 g./l.

DETAILED DESCRIPTION OF THE PREFERRED EMBODIMENTS

It has been found that by using both the polyoxyethylene compounds of the invention and the ketones of the invention in the presence of certain carboxylic acids, the bright plating current density range is considerably extended over that obtained when either the carboxylic acid or ketone compounds are omitted, in accordance with certain of the teachings of the prior art. Preferably two or more different molecular weights of the polyethylene compounds of the invention are used at the same time to obtain the most beneficial results and widest bright plating range.

The operating pH of the bath is established at about 3.5 to 6.1 because at a pH much below 3.5 undesirable dissolution of zinc anodes occurs even without electrolysis, and at a pH much above 6.1 precipitation of insoluble zinc salts commences. In operation, the bath tends to seek its own pH level of about 5.8 to 6.1, and lower pH levels can be maintained only by periodic additions of acid. The higher pH is also desirable in that it minimizes corrosion effects on plated parts due to poor rinsing.

While baths can be operated with the zinc metal content outside the preferred range of 30 to 60 g./l., such conditions are less preferred due to decreasing cathode efficiencies at lower zinc concentrations and increasing low current density dullness at higher concentrations.

The preferred range for total chloride ion content of 150 to 190 g./l. is arrived at from a recognition of the fact that baths containing lower concentrations of chloride, while operable, have the disadvantages of poorer low current density operation, poorer anode corrosion, and a tendency to precipitate insoluble zinc salts at pH's much above 5.5.

It should be recognized that bath formulations may also contain other metal salts such as, for example, potassium sulfate or sodium sulfamate. However, there appears to be little practical advantage to using such materials. Bath formulations may also contain mixtures of zinc salts such as zinc sulfate along with the zinc chloride. Again, there appears to be little or no practical advantage to this, and the preferred range of chloride content of the bath should still be met. If no zinc chloride is used, this chloride should come primarily from ammonium chloride. Alternative sources of zinc include zinc oxide dissolved in common industrial acids such as hydrochloric, sulfuric, acetic, fluoboric, and sulfamic acids. Alternatively, aqueous solutions of commercial zinc salts themselves may be employed, and, as mentioned above, zinc chloride is preferred.

The pH of the bath is adjusted to the desired level by means of addition of ammonium hydroxide, sodium hydroxide or equivalent materials.

The zinc electrode deposits obtained from such acid baths are typically coarse and dull in appearance and have little commercial value until other additives are used. The additive of the invention including certain nonionic polyoxyethylene compounds, certain ketones, and certain carboxylic acids, each component added to the bath in suitable amounts, permits the production of a bright, shiny zinc electrodeposit of a high decorative quality over a wide range of operating current densities and in a higher pH range than taught by the prior art.

As discussed above, the higher pH range is desirable.

Brightener chemicals are preferably added to the bath as two types of additives in order to obtain the correct balance of components for initial start up and subsequent continued maintenance of the bath under optimum conditions of performance.

A starter additive is usually used only once at the start as a new bath is made up. It comprises an aqueous solution containing: polyoxyethylene compounds: 100 to 500 g./l., preferably 200 to 350 g./l.; and carboxylic acid (added as sodium, potassium, ammonium or similar salts) 50 to 250 g./l., preferably 100 to 200 g./l.

A maintenance additive is added initially to the bath and then on demand to maintain performance. It comprises an organoaqueous solution containing: polyoxyethylene compounds 10-400 g./l. preferably 20 to 50 g./l.; carboxylic acid (as sodium, potassium, ammonium or similar salt) 10-200 g./l. preferably 20 to 50 g./l.; and ketone 10 to 200 g./l., preferably 20 to 50 g./l. In the maintenance additive, methanol is used to solubilize the sparingly soluble ketones of the invention. The amount of methanol required varies depending on the concentration of ketone used in the formulation, but typically may comprise 30 to 50 percent by weight of the formulation. In place of methanol other inexpensive organic solvents such as ethanol, acetone and the like may be employed.

In practicing the invention in the start up of a new bath, the desired amount of starter additive, typically 10 to 40 cc. per liter of bath, is added to the bath and well mixed. Next the desired amount of maintenance additive typically 10 to 40 cc. per liter of bath is added to the bath and well mixed. The bath is now ready for operation.

To illustrate the operation of the invention and its superiority over the prior art, the experiments were performed which are set forth in the following examples. In the examples, an aqueous bath containing 75 g./l.  $ZnCl_2$ , and 185 g./l.  $NH_4Cl$  was used. The temperature of operation was about 20°C. The pH and other parameters, and the additives used and their concentrations are stated in the examples, and the resulting characteristics of plates at various current densities are set forth. For the polyoxyethylene compounds, the approximate molar content of the polyoxyethylene is given.

EXAMPLE 1

50 Demonstrating Advantages of Three-Component Addition. Carboxylic Acid Omitted in First Test

Test 1: To 1 liter of zinc chloride/ammonium chloride bath, at pH 5.0, were added:

|                                                                                     |                  |
|-------------------------------------------------------------------------------------|------------------|
| $(polyoxyethylene)_{10, mol}$ tetramethyl decyn diol ("Surlynol 465")               | 2.0 g.           |
| $(polyoxyethylene)_{30, mol}$ tetramethyl decyn diol ("Surlynol 485") benzalacetone | 2.0 g.<br>0.2 g. |

60 267 ml. of this solution were transferred to a Hull cell and a steel cathode panel plated at 2 amps for 10 minutes. The panel showed the following plate characteristics:

|                           |                  |
|---------------------------|------------------|
| 0-10 a./ft. <sup>2</sup>  | dull, gray black |
| 10-14 a./ft. <sup>2</sup> | bright           |
| 14-20 a./ft. <sup>2</sup> | dull, gray       |

5

-Continued  
bright  
bright but very rough plate.

Test 2: To the same solution were next added 2 g. benzoic acid (as sodium salt). A repeat 2 a./10 min. Hull cell panel test now showed:

0-80 a./ft.<sup>2</sup>  
Above 80 a./ft.<sup>2</sup> very bright  
very bright but some roughness.

5

(polyoxyethylene)<sub>30</sub> mol tetramethyl  
decyn diol  
2-furanacrylic acid  
furfuralacetone

8.0 g.  
5.0 g.  
0.4 g.

6

A steel cathode plated at 2 amps for 10 minutes in a 267 ml. Hull cell gave:

0-60 a./ft.<sup>2</sup>  
60-100 a./ft.<sup>2</sup>  
above 100 a./ft.<sup>2</sup> very bright  
semibright, rough  
dull, black.

## EXAMPLE 2

Demonstrating Advantages of Three-Component System Carbonyl Compound Omitted in First Test

Test 1: To 1 liter of zinc chloride/ammonium chloride bath, at pH 5.5, were added:

(polyoxyethylene)<sub>10</sub> mol tetramethyl  
decyn diol 2.0 g.  
(polyoxyethylene)<sub>30</sub> mol tetramethyl  
decyn diol 2.0 g.  
benzoic acid (as sodium salt) 2.0 g.

A steel cathode panel plated at 2 amps for 10 minutes in a 267 ml. Hull cell showed the following plate characteristics:

0-1 a./ft.<sup>2</sup>  
1-35 a./ft.<sup>2</sup>  
above 35 a./ft.<sup>2</sup> dull, gray  
semibright  
dull, black.

Test 2: To the same solution were added 0.2 g. benzalacetone. A repeat, 2 a./10 min., Hull cell panel now showed:

0-80 a./ft.<sup>2</sup>  
above 80 a./ft.<sup>2</sup> very bright  
semibright, rough.

## EXAMPLE 3

Operation at pH 6

To 1 liter zinc chloride/ammonium chloride bath at pH 6.0 were added:

(polyoxyethylene)<sub>10</sub> mol tetramethyl  
decyn diol 2.0 g.  
(polyoxyethylene)<sub>30</sub> mol tetramethyl  
decyn diol 2.0 g.  
benzoic acid (as sodium salt) 2.0 g.  
benzalacetone 0.2 g.

A steel panel plated at 2 amps for 10 minutes in a 267 ml. Hull cell gave:

0-75 a./ft.<sup>2</sup>  
above 75 a./ft.<sup>2</sup> bright  
semibright, rough.

The brightness here was not quite that obtained in Examples 1 and 2. However, increasing the benzalacetone concentration to 0.3 g./l. fully restored the brightness level.

## EXAMPLE 4

To 1 liter zinc chloride/ammonium chloride bath at pH 5.3 were added:

15 15 To 1 liter zinc chloride/ammonium chloride bath at pH 5.4 were added:

20 (polyoxyethylene)<sub>22</sub> mol (polyoxypropylene  
glycol)<sub>18</sub> mol ("Pluronic F 88") 2.0 g.  
benzalacetone 0.3 g.  
nicotinic acid 4.0 g.

25 A 267 ml. steel Hull cell cathode plated at 2 amps for 10 minutes showed:

30 0-50 a./ft.<sup>2</sup>  
50-60 a./ft.<sup>2</sup>  
60-100 a./ft.<sup>2</sup>  
above 100 a./ft.<sup>2</sup> bright  
dull  
bright  
dull.

## EXAMPLE 5

35 To 1 liter zinc chloride/ammonium chloride bath at pH 5.1 were added:

40 (polyoxyethylene)<sub>22</sub> mol (polyoxypropylene  
glycol)<sub>18</sub> mol ("Pluronic L 35") 8.0 g.  
(polyoxyethylene)<sub>10</sub> mol tetramethyl  
decyn diol 0.75 g.  
(polyoxyethylene)<sub>30</sub> mol tetramethyl  
decyn diol 0.75 g.  
furfural acetone 1.5 g.  
nicotinic acid 1.0 g.

45 A steel Hull cell panel plated at 2 amps for 10 minutes gave a deposit which was brilliant over the current density range 0-120 a./ft.<sup>2</sup> except for some roughness and a few dull vertical streaks in the range 70-90 a./ft.<sup>2</sup>

## EXAMPLE 7

50 To 1 liter zinc chloride/ammonium chloride bath at pH 5.1 were added:

55 (polyoxyethylene)<sub>210</sub> mol N,N,N',N'-tetrakis(poly-  
propylene glycol)<sub>48</sub> mol ethylene diamine 4 g.  
benzoic acid 4 g.  
benzalacetone 0.2 g.

60 A steel Hull cell panel plated at 2 amps for 10 minutes gave a bright zinc deposit over the range 0-60 a./ft.<sup>2</sup>

## EXAMPLE 8

65 A 105 liter zinc chloride/ammonium chloride bath at pH 5.9 was prepared. To it as brightener were added:

|                                                            |           |
|------------------------------------------------------------|-----------|
| (polyoxyethylene) <sub>10</sub> mol tetramethyl decyn diol | 2.0 g./l. |
| (polyoxyethylene) <sub>30</sub> mol tetramethyl decyn diol | 2.0 g./l. |
| benzoic acid (as sodium salt)                              | 2.0 g./l. |
| benzalacetone                                              | 0.2 g./l. |

A variety of parts including nuts, bolts, washers, safety harness clamps were barrel plated in a horizontal barrel for 20-30 minutes. Loading varied from 900-1,800 grams and plating current from 20-45 amps. Bright, shiny, well-adherent zinc with good coverage in recesses was obtained on all parts.

Various other parts — radio speakers, radio chassis, chain, wheel rims were rack plated in the same bath using average current densities of 20-60 a./ft.<sup>2</sup> and air agitation. Again, bright, shiny, well-adherent zinc with good coverage in recesses was obtained on all parts.

I claim:

1. A composition for providing bright zinc electrode deposits which comprises an aqueous acidic electrolyte composition containing at least one zinc compound providing zinc ions for electroplating zinc, a source of chloride ion, 0.05 to 20 g./l. of at least one nonionic polyoxyethylene compound, 0.05 to 2 g./l. of at least one ketone, and 0.05 to 20 g./l. of at least one carboxylic acid,

said polyoxyethylene compound being selected from compounds of the formula:



wherein  $n + m \geq 10$ ,  $x = 1$  or  $2$ , derived from a reaction of oxyethylene with a polyol selected from the group consisting of 2,4,7,9-tetramethyl-5-decyne-4,7 diol, polyoxypropylene glycol of molecular weight at least about 900, and N,N,N',N'-tetrakis(polyoxypropylene glycol) ethylene diamine of molecular weight at least about 500, and wherein R is defined by the selected polyol;

said ketone being selected from the group consisting of 4-phenyl-3-buten-2-one, 4-(4-methoxyphenyl)-3-buten-2-one, 4-(3,4-dimethoxyphenyl)-3-buten-2-one, 4-(3,4-methylenedioxyphenyl)-3-buten-2-one, and 4-(2-furyl)-3-buten-2-one; and

said carboxylic acid being selected from the group consisting of benzoic acid, cinnamic acid, 2-furylacrylic acid, and nicotinic acid.

2. A composition according to claim 1 having a zinc metal content within the range of about 30 to 60 g./l. with the zinc added as zinc chloride, a total chloride ion content of about 150 to 190 g./l. with the chloride other than zinc chloride being added in the form of ammonium chloride, a pH in the range of about 3.5 to 6.1, the polyoxyethylene compounds being present in the range of about 0.05 to 20 g./l., the ketone being present

in the range of about 0.05 to 2 g./l., and the carboxylic acid being present in the range of about 0.05 to 20 g./l.

3. A composition according to claim 2 having a pH in the range of about 5 to 6, a content of polyoxyethylene compounds in the range of about 2 to 10 g./l., a ketone content of about 0.1 to 0.5 g./l., and a carboxylic acid content of about 1 to 6 g./l. wherein said polyoxyethylene compounds are polyoxyethylene 2,4,7,9-tetramethyl-5-decyne-4,7 diol and said ketone is 4-phenyl-3-buten-2-one.

4. A composition according to claim 1 wherein the polyol is 2,4,7,9-tetramethyl-5-decyne-4,7 diol.

5. A composition according to claim 1 wherein the polyol is polyoxypropylene glycol of molecular weight of at least 900.

6. A composition according to claim 1 wherein the polyol is N,N,N',N'-tetrakis(polyoxypropylene glycol) ethylene diamine of molecular weight at least about 500.

7. A composition according to claim 1 wherein said ketone is 4-phenyl-3-buten-2-one.

8. A composition according to claim 1 wherein said ketone is 4-(4-methoxyphenyl)-3-buten-2-one.

9. A composition according to claim 1 wherein said ketone is 4-(3,4-dimethoxyphenyl)-3-buten-2-one.

10. A composition according to claim 1 wherein said ketone is 4-(3,4-methylenedioxyphenyl)-3-buten-2-one.

11. A composition according to claim 1 wherein said ketone is 4-(2-furyl)-3-buten-2-one.

12. A composition according to claim 1 wherein said carboxylic acid is benzoic acid.

13. A composition according to claim 1 in which the pH is in the range of about 3.5 to 6.1.

14. A composition according to claim 1 wherein the zinc concentration measured as metal is in the range of about 30 to 60 g./l., and the zinc is provided as zinc chloride.

15. A composition according to claim 1 wherein the bath has a total chloride ion concentration of about 150 to 190 g./l., with the major portion of the chloride being provided as zinc chloride and ammonium chloride.

16. A composition according to claim 1 wherein the polyoxyethylene compounds are present in a concentration range of about 2 to 10 g./l.

17. A composition according to claim 1 wherein the ketone is present in concentration range of about 0.1 to 0.5 g./l.

18. A composition according to claim 1 wherein the carboxylic acid is present in a concentration range of about 1 to 6 g./l.

19. A method of producing bright zinc electrodeposits which comprises passing current from an anode to a cathode at a temperature about in the range of 15° to 40°C. through an aqueous acidic electrolyte composition containing at least one zinc compound providing zinc ions for electroplating zinc, a source of chloride ion, 0.05 to 20 g./l. of at least one nonionic polyoxyethylene compound, 0.05 to 2 g./l. of at least one ketone, and 0.05 to 20 g./l. of at least one carboxylic acid, said polyoxyethylene compound being selected from compounds of the formula



wherein  $n + m \geq 10$ ,  $x = 1$  or  $2$ , derived from a reaction of oxyethylene with a polyol selected from the group consisting of 2,4,7,9-tetramethyl-5-decyne-4,7 diol, polyoxypropylene glycol of molecular weight at least about 900, and N,N,N',N'-tetrakis(polyoxypropylene glycol) ethylene diamine of molecular weight at least about 500,

and wherein R is defined by the selected polyol; said ketone being selected from the group consisting of

4-phenyl-3-buten-2-one,  
4-(4-methoxyphenyl)-3-buten-2-one,  
4-(3,4-dimethoxyphenyl)-3-buten-2-one,  
4-(3,4-methylenedioxophenyl)-3-buten-2-one, and  
4-(2-furyl)-3-buten-2-one; and

said carboxylic acid being selected from the group consisting of benzoic acid, cinnamic acid, 2-furylacrylic acid, and nicotinic acid.

20. A method of claim 19 operated at temperatures in the range of 15° to 40°C. with a zinc metal content within the range of about 30 to 60 g./l., the zinc being added as zinc chloride, a total chloride ion content of about 150 to 190 g./l. with the chloride other than zinc chloride being added in the form of ammonium chloride, a pH in the range of about 3.5 to 6.1, the polyoxyethylene compounds being present in the range of about 0.05 to 20 g./l., the ketone being present in the range of about 0.05 to 2 g./l., and the carboxylic acid being present in the range of about 0.05 to 20 g./l.

21. A method of claim 20 having a pH in the range of about 5 to 6, a content of polyoxyethylene compounds in the range of about 2 to 10 g./l., a ketone content of about 0.1 to 0.5 g./l., and a carboxylic acid content of about 1 to 6 g./l. wherein said polyoxyethylene compounds are polyoxyethylene 2,4,7,9-tetramethyl-5-decyne-4,7 diol and said ketone is 4-phenyl-3-buten-2-one.

22. A method of claim 19 wherein the pH is in the range of about 3.5 to 6.1.

23. A method of claim 19 wherein the zinc concentration measured as metal is in the range of about 30 to 60 g./l., and the zinc is provided as zinc chloride.

24. A method of claim 19 wherein the bath has a total chloride ion concentration of about 150 to 190 g./l., with the major portion of the chloride being provided as zinc chloride and ammonium chloride.

25. A method of claim 19 wherein the polyoxyethylene compounds are present in a concentration range of about 2 to 10 g./l.

26. A method of claim 19 wherein the ketone is present in a concentration range of about 0.1 to 0.5 g./l.

27. A method of claim 19 wherein the carboxylic acid is present in a concentration range of about 1 to 6 g./l.

10 28. An organoaqueous addition agent for use in preparing an acid zinc electroplating bath composition, said addition agent comprising:

10 to 400 g./l. of at least one nonionic polyoxyethylene compound selected from the group consisting of



wherein  $n + m \geq 10$ ,  $x = 1$  or  $2$ , derived from a reaction of oxyethylene with a polyol selected from the group consisting of

2,4,7,9-tetramethyl-5-decyne-4,7 diol, polyoxypropylene glycol of molecular weight at least about 900, and

N,N,N',N'-tetrakis(polyoxypropylene glycol) ethylene diamine of molecular weight at least about 500,

and wherein R is defined by the selected polyol; 10 to 200 g./l. of a ketone selected from the group consisting of

4-phenyl-3-buten-2-one,  
4-(4-methoxyphenyl)-3-buten-2-one,  
4-(3,4-dimethoxyphenyl)-3-buten-2-one,  
4-(3,4-methylenedioxophenyl)-3-buten-2-one, and  
4-(2-furyl)-3-buten-2-one; and

10 to 200 g./l. of a carboxylic acid selected from the group consisting of benzoic acid, cinnamic acid, 2-furylacrylic acid, and nicotinic acid.

29. An addition agent according to claim 28 wherein the polyoxyethylene compounds are polyoxyethylene 2,4,7,9-tetramethyl-5-decyne-4,7 diols, the ketone is 4-phenyl-3-buten-2-one, and the carboxylic acid is benzoic acid.

30. An addition agent according to claim 29 containing 20 to 50 g./l. of the polyoxyethylene compounds, 20 to 50 g./l. of the ketone, and 20 to 50 g./l. of the carboxylic acid.

\* \* \* \* \*

UNITED STATES PATENT OFFICE  
CERTIFICATE OF CORRECTION

PATENT NO. : 3,855,085  
DATED : December 17, 1974  
INVENTOR(S) : John Derek Rushmere

It is certified that error appears in the above-identified patent and that said Letters Patent are hereby corrected as shown below:

Column 9, line 5, "wherein  $n + m \cdot 10$ ," should be  
-- wherein  $n + m \geq 10$ , --.

Signed and Sealed this  
fifth Day of August 1975

[SEAL]

Attest:

**RUTH C. MASON**  
*Attesting Officer*

**C. MARSHALL DANN**  
*Commissioner of Patents and Trademarks*